

## UNITED STATES PATENT OFFICE

JOHN ALLEN HIGGINS, OF ST. JOSEPH, MISSOURI, ASSIGNOR TO EMMA HIGGINS,  
OF ST. JOSEPH, MISSOURI

## COMPOSITE LUBRICANT

No Drawing.

Application filed March 3, 1927. Serial No. 172,572.

This invention relates to lubricants and particularly to composite lubricants containing mineral and vegetable oils.

The principal object of my invention is to provide a composite lubricant containing mineral and vegetable oils so blended as to form a stable, homogeneous composition of high lubricating efficiency and whose viscosity is maintained to a very unusual degree during prolonged use even under conditions highly unfavorable to the action of ordinary lubricants.

Another object of this invention is to provide a composite lubricant which will maintain its lubricity substantially unimpaired at high temperatures and which will not "gum" at either unusually high or low temperatures.

A further object of the invention is to provide a lubricant which will not exercise a corrosive action by the decomposition of oils into fatty or other acids under any condition of use to which the lubricant is intended to be put.

A further object of the invention is to provide a lubricant which in addition to its lubricating properties exercises a detergent action on metals with which it comes into contact thereby preventing to a considerable extent the accumulation of dirt or other foreign matter thereon and effecting or facilitating its removal if already formed.

Other objects and advantages will be apparent in the course of the following description.

Mineral oils and vegetable oils each have their individual merits or advantages as lubricants. Many attempts have been made to provide lubricants containing both mineral and vegetable oils which would be superior to either. These efforts have however, met with but indifferent success commercially owing to the use in the production of the mixtures of chemicals injurious to the parts to be lubricated or to the mixtures being unstable or otherwise unsatisfactory or to the excessive cost of producing a satisfactory blend of such oils or for other reasons.

I have found that a stable composite lubricant having the advantages hereinbefore set forth in the statement of objects of this in-

vention may be obtained by the employment of petroleum and vegetable oils blended or united as hereinafter described.

In the preferred process of producing my composite lubricant I first produce what I term "mixture No. 1" by dissolving 1 pound of caoutchouc preferably of the grade known as fresh smoke sheet caoutchouc, in a suitable solvent of caoutchouc, preferably benzine or high test gasoline, using only a sufficient quantity of the solvent to produce a complete solution of the caoutchouc. Using fresh high grade caoutchouc 3 quarts of high test gasoline is preferably employed in making the solution. I then add this solution to from 15 to 50 gallons, preferably about 25 gallons, of mineral oil preferably a neutral high grade lubricating oil of the character commonly used in automobile lubrication. I prefer to employ an oil of light or medium viscosity but a heavy or even an extra heavy oil may be used. The mixture is stirred thoroughly and allowed to stand for preferably about 36 hours. To this mixture I then add preferably about 8 to 10 ounces of cocoanut oil and stir thoroughly.

I then produce what I term "mixture No. 2" by mixing 50 gallons of castor oil preferably of the grade known as No. 2 castor oil, with 50 gallons of another vegetable seed oil such as cottonseed oil or rape seed oil, but preferably high grade water white cottonseed oil. Although rape seed oil readily blends with castor oil and is suitable for use therewith in the practice of my invention its high cost renders its use less advantageous than the use of cottonseed oil which is relatively inexpensive. The mixture is heated preferably slowly to about 160° F. while being stirred. The heating is then discontinued and the mixture allowed to stand for about 48 hours.

To 100 gallons of mineral lubricating oil I add from 1 to 10 per cent. preferably about 8 per cent. by volume of mixture No. 1 and the same amount of mixture No. 2. This final mixture is then heated preferably slowly to about 150° F. while being stirred. It is then allowed to cool and is ready for use. In this final operation I may use any mineral lubricating oil from a light spindle oil to extra

heavy lubricating oil depending upon the use for which my composite lubricant is intended. I may even employ the highly viscous mineral oils commonly known as greases if a very viscous lubricant is desired as for example, for use in grease cups.

From the foregoing it will be apparent that the composite lubricant produced in accordance with the preferred practice of my process will contain the following ingredients in approximately the following proportions: 102 gallons of mineral lubricating oil, .64 to .8 of an ounce of cocoanut oil, .8 of a pound of caoutchouc, 4 gallons of castor oil, and 15 4 gallons of white cottonseed oil.

I have found that I can produce a serviceable and efficient stable composite lubricant without the use of castor oil by the following modification in my composition and process:

20 To 100 gallons of a mineral oil I add from 1 to 10 per cent., preferably about 8 per cent. of a vegetable seed oil preferably high grade water white cottonseed oil and the same amount of mixture No. 1 above referred to.

25 This mixture is heated preferably slowly to about 150° F. while being stirred. It is then allowed to cool and is ready for use.

The solvent used in dissolving the caoutchouc is largely driven off in the heating operation and is not present at least to any considerable extent, in the finished product. I may in fact, produce a fairly stable composite lubricant containing both mineral and vegetable oils without the use of the dissolved caoutchouc in which case I employ only the mineral oil and cocoanut oil in the preferred proportions indicated in making mixture No. 1. Even the small proportion of the cocoanut oil used is sufficient to affect the 40 blending of the mineral and vegetable oils into a homogeneous and fairly stable mixture. I prefer however to employ the caoutchouc as well as the cocoanut oil in my composition since an entirely stable blend is produced in 45 such case and the finished product is found to be in other respects a more satisfactory one.

It will be understood that the examples given are merely illustrative of the preferred 50 embodiment of my composition and process of producing it. The proportions and details of procedure may be widely varied and meritorious results obtained but the best results have been obtained by proceeding as described and employing the ingredients in the proportions indicated.

In dissolving the caoutchouc I have found that it is not necessary to wholly dissolve it 55 in the solvent. I may advantageously cut the caoutchouc into small pieces and add only sufficient of the solvent to partially dissolve it. The pieces of caoutchouc under the action of the solvent swell and assume a pasty form and this may be employed instead of a com-

plete solution, the mass being finally completely dissolved in mixture No. 1.

70 My composite lubricant is adapted for advantageous use for all lubricating purposes except in contact with steam as in the lubrication of steam engine cylinders and for such use it is not recommended. It is however, particularly advantageous for use in aeroplane and other high duty internal combustion engines and for other lubrication where 75 only the highest grade and most expensive lubricants heretofore have been successfully employed.

80 My composition is inexpensive to produce and economical in use its lubricating efficiency being maintained for unusually long periods even under conditions highly unfavorable to the life of lubricating compositions.

85 While I have described in detail the preferred embodiment and practice of my invention it is to be understood that it is not restricted thereto except as set forth in the appended claims.

90 Having described my invention, I claim:

1. A composite lubricant comprising a mineral lubricating oil, cocoanut oil, cottonseed oil, castor oil, and caoutchouc in the approximate proportions of 102 gallons of the mineral oil, .64 to .8 of an ounce of the cocoanut oil, 4 gallons of the cottonseed oil, 4 gallons of the castor oil, and .8 of a pound of the caoutchouc.

95 2. A composite lubricant comprising a mixture of substantially one pound of caoutchouc 100 dissolved in gasoline, substantially twenty-five gallons of a neutral mineral lubricating oil and approximately eight ounces of cocoanut oil, added to and mixed with substantially fifty gallons of castor oil having substantially 105 fifty gallons of cotton seed oil mixed therewith.

3. A composite lubricant comprising a mixture of caoutchouc dissolved in gasoline, a neutral mineral lubricating oil, and cocoanut oil, added to and mixed with castor oil 110 having cotton seed oil mixed therewith.

In testimonay whereof I affix my signature.  
JOHN ALLEN HIGGINS.

115

120

125

130